# EUROPEAN PATENT SPECIFICATION

(11) **EP 0 830 257 B1**
(45) Date of publication and mention of the grant of the patent: **21.04.1999**
(21) Application number: 96916231.2
(22) Date of filing: 04.06.1996
(51) Int. Cl.: B41M 5/00, D21H 19/22

(54) **Natural tracing paper for use with pigment-based inks.**
Natürliches Pauspapier für die Verwendung von Farbstoffen.
Papier à calquer naturel destiné à être utilisé avec des encres à base de pigments.

(30) Priority: 06.06.1995 GB 9511363
(43) Date of publication of application: 25.03.1998
(73) Proprietor: Rexam Coated Products Limited, London SW1 X7N (GB)
(72) Inventor: BODY, James, Christopher, Canterbury CT4 7JA (GB); BRACEWELL, Robert, Graham, Canterbury CT4 7JA (GB); OWEN, Peter, Kevin, Canterbury CT4 7JA (GB)
(74) Representative: Raynor, Simon Mark
(86) International application number: GB9601326
(87) International publication number: WO9639304

(56) References cited:
- EP-A- 0 495 430
- EP-A- 0 514 633
- EP-A- 0 524 635
- EP-A- 0 582 466
- EP-A- 0 631 881
- GB-A- 2 213 078

## Description

The present invention relates to a natural tracing paper for use with ink-jet printers and plotters employing pigment-based inks.

Natural tracing paper (as opposed to "prepared" tracing paper, also known as "vellum") is manufactured from wood-based cellulose fibre pulp, which is mechanically treated, for example by crushing and chopping, to remove any air/fibre interfaces. This renders the paper material translucent. The finished tracing paper is relatively dense and impervious compared with normal opaque papers.

EP-A-0631881 describes an opaque printing material comprising a support and an ink receiving layer containing a pigment, a hydrophilic binder and a quaternary ammonium compound.

Tracing papers have been used for many years for the preparation of engineering master drawings to be reproduced by the diazo process. Although manual drafting has largely been superseded by the use of CAD systems, tracing papers are still used for printing the master drawings. Various types of plotter are used for printing the drawings, including pen plotters and electrostatic printers, but one of the most favoured types of plotter at present is the ink jet plotter.

Some ink jet print heads available at present use dye-based inks. These are satisfactory for most general purpose applications such as printing text and some graphic material, but lack the density and permanence of the pigment-based inks that have traditionally been used in the preparation of engineering master drawings. The lower density of the ink means that drawings printed using dye-based inks are not as well suited to the diazo process as those produced using pigment based inks.

More recently, an ink-jet print head that uses pigment-based inks has become available. This print head produces denser images than the previous dye-based ink print heads and the resulting drawings are better adapted to the diazo copying process. The images are also less liable to fading than images produced using dye-based inks.

The development of the new ink jet print head has required the parallel development of new types of pigment-based ink. As the speed and definition of the print head has increased, the formulations of these new inks have been revised to provide the necessary performance.

A pigment-based ink for use with an ink jet print head typically comprises a dispersion of pigment particles, such as carbon black, suspended within an aqueous vehicle. Other ingredients, such as surfactants and stabilizers, are usually included to help maintain the dispersion, to prevent blocking of the ink jet nozzles and to promote vaporisation of the ink in the print head. However, unlike traditional pigment-based inks such as Indian ink, a binder such as shellac is not generally included as this can lead to blocking of the ink jet nozzles.

The applicants have identified a problem with existing tracing papers when used with ink jet print heads employing pigment-based inks. This is that when relatively large blocks or areas (i.e. areas larger than a few mm²) of high density are printed, the print can become rather uneven. For example, the print density may be reduced towards the edges of the area and stripes or patches of varying density may be produced. This phenomenon is sometimes referred to as "cascading". The variations in density are particularly noticeable by transmitted light and they can, therefore, be transferred to copies made by the diazo process. The effect is not generally particularly noticeable by reflected light or in areas of text or fine details.

The applicants have observed that the above-mentioned problem occurs when the ink droplets fall onto the paper in such a concentration that they coalesce to form a pool of liquid ink on the surface of the paper. The applicants have discovered that when this happens, the pigment particles migrate towards one another within the pool of liquid, thereby forming areas of increased density and leaving areas of reduced density.

A similar problem has been observed with colour print heads that use pigment-based black ink and dye-based coloured inks. Where an area of pigment-based ink touches an area of dye-based ink, the border between the two inks becomes scalloped with the coloured dye-based inks intruding into the black area. The applicants have discovered that this effect is caused by migration of the pigment particles away from the area of dye-based ink.

It is an object of the invention to provide a natural tracing paper that mitigates at least some of the above-mentioned problems.

According to a first aspect of the invention there is provided a natural tracing paper for use with ink-jet printing using pigment-based inks, said natural tracing paper comprising a paper manufactured from a wood-based cellulose fibre pulp that is mechanically treated to render the paper translucent, wherein at least a usable surface of the natural tracing paper includes a combination of a water soluble cationic substance and water soluble binder substance.

In experiments involving the application of various surface treatments to the tracing paper, the applicants found that by treating the surface of the sheet with a water soluble cationic substance, the suspension of pigment particles could be destabilized as the ink droplets hit the surface, giving good print quality. However, abrasion resistance of the print was unsatisfactory. The printed documents did not, therefore, have the longevity required of them. The applicants discovered that this was because the pigment particles tended to sit on the surface of the paper, where they were exposed to abrasive forces, rather than being drawn into the structure of the paper.

The applicants have further found, however, that if the surface of the tracing paper is also treated with a water soluble or water-swellable binder, the resistance of the ink to abrasion is greatly increased. Therefore, by treating the tracing paper with a binder substance in combination with a cationic substance, migration can be largely prevented and the print quality and permanence of the printed sheet thereby improved.

The cationic substance may be a soluble polyvalent metal salt. Suitable metal salts include the salts of metals from Groups II and III or the Transition Metals of the Periodic Table. Preferably, the metal salt is a salt of a cation selected from the group consisting of Mg²⁺, Ca²⁺, Al³⁺, Zr⁴⁺ and Zn²⁺. Examples of suitable metal salts include magnesium sulphate, calcium chloride, ammonium sulphate, zinc acetate, ammonium zirconium carbonate and magnesium acetate.

Alternatively, the cationic substance may be a cationic polymer, and is preferably a low molecular weight, high cationic charge density, water soluble organic polymer. For example, the polymer may be a polymeric amine (such as a quaternary amine or easily protonated tertiary amine). A suitable cationic substance is a solution in water of a poly-quaternary amine.

The binder substance may be selected from a group consisting of polyvinylpyrrolidone (PVP), polyvinyl alcohol (PVOH), carboxylated cellulosic polymers, polyacrylic acids, hydroxylated polyacrylates, polyacrylamides, starches (for example oxidised potato starch and potato starch ethers) and gelatine (compounded animal protein in water).

Examples of suitable carboxylated cellulosic polymers include carboxyalkyl polymers and hydroxyalkyl polymers, and preferably hydroxymethyl cellulose and hydroxypropyl cellulose, and more preferably carboxymethylcellulose (CMC) (especially low molecular weight carboxymethylcellulose).

Examples of suitable polyacrylic acids include those sold under the Trade Marks POLYMIN SK, PERCOL 1597 and PERCOL 1697.

Various types of polyvinyl alcohol (PVOH) may be used, including those having a low hydrolysis level and a high molecular weight, a low hydrolysis level and a low molecular weight, a high hydrolysis level and a high molecular weight, or a high hydrolysis level and a low molecular weight. The binder substance may have a molecular weight in the range 790,000 to 1,350,000 and a viscosity defined by a K-value of at least 30, and preferably at least 60, and advantageously approximately 90.

In a particularly preferred embodiment of the invention, the cationic substance is magnesium sulphate and the binder is PVP. The amount of magnesium sulphate applied to the surface of the tracing paper is preferably in the range 0.5-3.0gm⁻², and more preferably 1.0-2.0gm⁻², and advantageously approximately 1.25-1.75gm⁻². The amount of PVP applied to the surface of the tracing paper is preferably in the range 0.15-0.75gm⁻², and more preferably 0.4-0.7gm⁻², and is advantageously approximately 0.5gm⁻².

The natural tracing paper is preferably an uncoated cellulose-based paper.

According to a second aspect of the invention, there is provided a method of manufacturing a natural tracing paper for use with an ink jet plotter or printer using pigment-based ink, said natural tracing paper comprising a paper manufactured from a wood-based cellulose fibre pulp that is mechanically treated to render the paper translucent, wherein at least a usable surface of the recording sheet is treated with a combination of a water soluble cationic substance and water soluble binder substance.

The tracing paper is advantageously treated by applying a solution of the combination of substances to the usable surface of the paper. Preferably, the solution is applied by drawing the semi-manufactured paper through a bath of the solution. Alternatively, the solution may be applied to the paper by spraying or coating, either during or after completion of the manufacturing process.

According to a third aspect of the invention, there is provided a method of printing in which a pigment-based ink is applied to a natural tracing paper with an ink-jet plotter or printer, said natural tracing paper comprising a paper manufactured from a wood-based cellulose fibre pulp that is mechanically treated to render the paper translucent, wherein at least a usable surface of the natural tracing paper includes a combination of a water soluble cationic substance and water soluble binder substance.

Various embodiments of the invention will now be described by way of the following examples, in which all parts and percentages are by weight unless otherwise stated.

### Examples

The effect of applying various substances to natural tracing paper was tested by applying the substances as aqueous solutions to a base paper comprising a 90gm⁻² waterleaf natural tracing paper. The effectiveness of the substances in reducing migration was assessed visually and the substances were ranked according to the categories excellent, fair, mediocre and poor (in descending order). The effectiveness of the substances in binding the printed image to the paper was tested by visually assessing the results of an abrasion test and the substances ranked according to the same categories.

The results of the tests are summarised in the following table (Table 1).

The tests revealed that whilst treating the surface of the paper with a cationic substance alone helps to reduce migration, this leads to poor resistance to abrasion. In order to provide good abrasion resistance as well as reduced migration, a binder must be applied in addition to the cationic substance. It was found that an aqueous solution comprising a blend of magnesium sulphate and high viscosity PVP produced excellent results, both for reducing migration and providing good resistance to abrasion.

**Table 1**

| Test results. | | | | | |
|---|---|---|---|---|---|
| Solution content | Class | Blend | Applied weight | Binding rating | Migration rating |
| Aluminium sulphate | Cation | no | 8.0 gm⁻² | poor | excellent |
| | | | 1.1 gm⁻² | poor | fair |
| Calcium chloride | Cation | no | 1.1 gm⁻² | poor | good |
| | | | 8.9 gm⁻² | poor | excellent |
| Magnesium sulphate | Cation | no | 1.0 gm⁻² | poor | good |
| | | | 8.5 gm⁻² | poor | excellent |
| Polymeric quaternary amine | Cation | no | 1.0 gm⁻² | poor | fair |
| | | | 11.1gm⁻² | poor | fair |
| Oxidised potato starch | Binder | no | 5.9 gm⁻² | fair | poor |
| | | | 1.2 gm⁻² | poor | poor |
| Potato starch ethers | Binder | no | 1.5 gm⁻² | poor | poor |
| | | | 3.6 gm⁻² | fair | poor |
| Polyvinyl alcohol (High hydrolysis, Low mol wt) | Binder | no | 1.0 gm⁻² | fair | poor |
| | | | 2.3 gm⁻² | fair | poor |
| Polyvinyl alcohol (Low hydrolysis, Low mol wt) | Binder | no | 1.0 gm⁻² | excellent | poor |
| | | | 2.3 gm⁻² | excellent | poor |
| Polyvinyl alcohol (High hydrolysis, High mol wt) | Binder | no | 0.4 gm⁻² | excellent | poor |
| | | | 0.8 gm⁻² | excellent | poor |
| Polyvinyl alcohol (Low hydrolysis, High mol wt) | Binder | no | 0.4 gm⁻² | mediocre | poor |
| | | | 1.3 gm⁻² | mediocre | poor |
| Low viscosity PVP | Binder | no | 0.1 gm⁻² | excellent | poor |
| | | | 0.5 gm⁻² | excellent | poor |
| Low viscosity CMC | Binder | no | 0.4 gm⁻² | fair | poor |
| | | | 0.1 gm⁻² | fair | poor |
| High viscosity PVP | Binder | yes | 0.2 gm⁻² | excellent | excellent |
| Magnesium sulphate | Cation | | 1.0 gm⁻² | excellent | excellent |
| High viscosity PVP | Binder | yes | 0.1 gm⁻² | excellent | excellent |
| Magnesium sulphate | Cation | | 0.9 gm⁻² | excellent | excellent |

## Claims

1. A natural tracing paper for ink-jet printing using pigment-based inks, said natural tracing paper comprising a paper manufactured from a wood-based cellulose fibre pulp that is mechanically treated to render the paper translucent, characterised in that at least a usable surface of the tracing paper includes a combination of a water soluble cationic substance and water soluble binder substance.

2. A natural tracing paper according to claim 1, wherein the cationic substance is a soluble polyvalent metal salt; and advantageously a salt of a metal from Groups II and III or the Transition Metals of the Periodic Table; and preferably a salt of a cation selected from the group consisting of Mg²⁺, Ca²⁺, Al³⁺, Zr⁴⁺ and Zn²⁺.

3. A natural tracing paper according to claim 2, wherein the cationic substance is magnesium sulphate.

4. A natural tracing paper according to claim 3, wherein the amount of magnesium sulphate applied to the surface of the natural tracing paper is in the range 0.5-3.0gm⁻², and preferably 1.0-2.0gm⁻², and advantageously approximately 1.25-1.75gm⁻².

5. A natural tracing paper according to claim 1, wherein the cationic substance is a cationic polymer; and advantageously a poly-quaternary amine.

6. A natural tracing paper according to any one of the preceding claims, wherein the binder substance is selected from a group consisting of polyvinylpyrrolidone, polyvinyl alcohol, carboxylated cellulosic polymers, polyacrylic acids, hydroxylated polyacrylates, polyacrylamides, starches and gelatine; and advantageously from a group consisting of carboxyalkyl polymers and hydroxyalkyl polymers; and preferably hydroxymethyl cellulose and hydroxypropyl cellulose, and more preferably carboxymethyl cellulose.

7. A natural tracing paper according to claim 6, wherein the binder substance has a molecular weight in the range 790,000 to 1,350,000.

8. A natural tracing paper according to claim 7, wherein the binder substance is polyvinylpyrrolidone having a viscosity defined by a K-value of at least 30, and preferably at least 60 and advantageously approximately 90.

9. A natural tracing paper according to claim 8, wherein the amount of PVP applied to the surface of the natural tracing paper is in the range 0.15-0.75gm⁻², and preferably 0.4-0.7gm⁻², and is advantageously approximately 0.5gm⁻².

10. A natural tracing paper according to any one of the preceding claims, in which the substances are applied to the surface of the natural tracing paper as an aqueous solution.

11. A method of manufacturing a natural tracing paper for use with an ink jet plotter or printer using pigment-based inks, said natural tracing paper comprising a paper manufactured from a wood-based cellulose fibre pulp that is mechanically treated to render the paper translucent, characterised in that at least a usable surface of the natural tracing paper is treated with a combination of a water soluble cationic substance and water soluble binder substance.

12. A method according to claim 11, wherein the natural tracing paper is treated by applying an aqueous solution of the combination of substances to the usable surface of the paper, advantageously by drawing the semi-manufactured natural tracing paper through a bath of the solution.

13. A method of printing, in which a pigment-based ink is applied to a natural tracing paper with an ink jet plotter or printer, said natural tracing paper comprising a paper manufactured from a wood-based cellulose fibre pulp that is mechanically treated to render the paper translucent, characterised in that at least a usable surface of the natural tracing paper includes a combination of a water soluble cationic substance and water soluble binder substance.

## Patentansprüche

1. Natürliches Pauspapier für das Farbstoff- oder Tintenstrahl-Drucken unter Verwendung von Farbstoffen oder Tinten auf Farbpigmentbasis, bestehend aus einem Papier, das aus Zellulosefaser-Pulpe auf Holzbasis hergestellt ist, die mechanisch bearbeitet wurde, um das Papier transparent zu machen, dadurch gekennzeichnet, daß wenigstens eine nutzbare Fläche des Pauspapieres eine Kombination einer wasserlöslichen kationischen Substanz und eines wasserlöslichen Bindemittels enthält.

2. Natürliches Pauspapier nach Anspruch 1, wobei die kationische Substanz ein lösliches mehrwertiges Metallsalz und vorteilhaft ein Salz eines Metalles aus der Gruppe II und III oder der Übergangsmetalle des Periodensystemes ist, und vorzugsweise ein Salz eines Kationes, das aus der Gruppe von MG²⁺, Ca²⁺, AL³⁺, ZR⁴⁺ und ZN²⁺ ausgewählt wurde.

3. Natürliches Pauspapier nach Anspruch 2, wobei die kationische Substanz Magnesiumsulfat ist.

4. Natürliches Pauspapier nach Anspruch 3, wobei die auf die Fläche des natürlichen Pauspapieres aufgebrachte Menge an Magnesiumsulfat im Bereich von 0,5-3,0 gm⁻² liegt und vorzugsweise im Bereich von 1,0-2,0 gm⁻², und vorteilhaft etwa im Bereich zwischen 1,25-1,75 gm⁻².

5. Natürliches Pauspapier nach Anspruch 1, wobei die kationische Substanz ein kationisches Polymer und vorteilhaft ein polyquaternäres Amin ist.

6. Natürliches Pauspapier nach einem der vorhergehenden Ansprüche, wobei das Bindemittel aus der Gruppe ausgewählt ist, die aus Polyvinylpyrrolidon, Polyvinylalkohol, Karboxyl-Cellulosepolymere, Polyacrylsäuren, Hydroxyl-Polyacrylate, Polyacrylamide, Stärken und Gelatine besteht, und vorteilhaft aus der Gruppe, die aus Karboxyalkyl-Polymeren und Hydroxyalkyl-Polymeren besteht, und vorzugsweise aus Hydroxymethylcellulose und Hydroxypropylcellulose, und noch stärker bevorzugt aus Karboxymethylcellulose.

7. Natürliches Pauspapier nach Anspruch 6, wobei das Bindemittel ein Molekulargewicht im Bereich von 790,000 bis 1,350,000 aufweist.

8. Natürliches Pauspapier nach Anspruch 7, wobei das Bindemittel ein Polyvinylpyrrolidon mit einer Viskosität ist, die durch einen K-Wert von mindestens 30, und vorzugsweise mindestens 60 und vorteilhaft von etwa 90 definiert ist.

9. Natürliches Pauspapier nach Anspruch 8, wobei die Menge an auf die Oberfläche des natürlichen Pauspapieres aufgebrachtem PVP (Polyvinylpyrrolidon) im Bereich von 0,15-075 gm⁻², und vorzugsweise im Bereich von 0,4-0,7 gm⁻² und vorteilhaft bei etwa 0,5 gm⁻² liegt.

10. Natürliches Pauspapier nach einem der vorhergehenden Ansprüche, wobei die Substanzen auf die Fläche des natürlichen Pauspapieres als wässerige Lösung aufgebracht werden.

11. Verfahren zum Herstellen eines natürlichen Pauspapieres für die Verwendung bei einem Tintenstrahl-Plotter oder - Drucker unter Verwendung von Farbstoffen oder Tinten auf Farbpigmentbasis, wobei das natürliche Pauspapier ein Papier enthält, das aus einer Zellulosefaser-Pulpe auf Holzbasis hergestellt ist, die mechanisch behandelt wurde, um das Papier transparent zu machen, dadurch gekennzeichnet, daß wenigstens eine nutzbare Fläche des natürlichen Pauspapieres durch eine Kombination einer wasserloslichen kationischen Substanz und eines wasserlöslichen Bindemittels behandelt wurde.

12. Verfahren nach Anspruch 11, wobei das natürliche Pauspapier durch Aufbringen einer Wässrigen Lösung aus einer Kombination von Substanzen auf die nutzbare Fläche des Papieres behandelt wird, vorzugsweise durch das Ziehen des halb fertig gestellten natürlichen Pauspapieres durch ein Bad der Lösung.

13. Verfahren zum Drucken, bei dem ein Farbstoff oder eine Tinte durch einen Farbstoff- oder Tintenstrahl-Plotter oder - Drucker auf das natürliche Pauspapier aufgebracht wird, wobei das natürliche Pauspapier aus einem Papier besteht, das aus einer Zellulosefaser-Pulpe auf Holzbasis hergestellt wurde, die mechanisch behandelt wurde, um das Papier transparent zu machen, dadurch gekennzeichnet, daß wenigstens eine nutzbare Fläche des natürlichen Pauspapieres eine Kombination einer wasserlöslichen kationischen Substanz und eines wasserlöslichen Bindemittels enthält.

## Revendications

1. Papier calque naturel susceptible d'être utilisé en impression à jet d'encre en utilisant des encres a base de pigments, ledit papier calque naturel comprenant un papier fabriqué à partir d'une pâte de fibres de cellulose à base de bois qui est mécaniquement traitée pour rendre le papier translucide, caractérisé en ce qu'au moins une surface utile du papier calque comprend une combinaison d'une substance cationique soluble dans l'eau et d'une substance liante soluble dans l'eau.

2. Papier calque naturel selon la revendication 1, dans lequel la substance cationique est un sel de métal polyvalent soluble et avantageusement un sel d'un métal des groupes II et III ou des métaux de transition du tableau périodique, de préférence un sel d'un cation choisi dans le groupe comprenant Mg²⁺, Ca²⁺, Al³⁺, Zr⁴⁺ et Zn²⁺.

3. Papier calque naturel selon la revendication 2, dans lequel la substance cationique est le sulfate de magnésium.

4. Papier calque naturel selon la revendication 3, dans lequel la quantité de sulfate de magnésium appliquée à la surface du papier calque naturel se situe dans la plage de 0,5 à 3,0 gm⁻², de préférence de 1,0 à 2,0 gm⁻², avantageusement d'environ 1,25 à 1,75 gm⁻².

5. Papier calque naturel selon la revendication 1, dans lequel la substance cationique est un polymère cationique et avantageusement une amine polyquaternaire.

6. Papier calque naturel selon l'une quelconque des revendications précédente, dans lequel la substance liante est choisie dans un groupe comprenant la polyvinylpyrrolidone, l'alcool polyvinylique, des polymères cellulosiques carboxylés, des acides polyacryliques, des polyacrylates hydroxylés, des polyacrylamides, des amidons et de la gélatine, et avantageusement dans un groupe comprenant des polymères carboxyalkylés et des polymères hydroxyalkylés, de préférence l'hydroxyméthylcellulose et l'hydroxypropylcellulose, mieux encore la carboxyméthylcellulose.

7. Papier calque naturel selon la revendication 6, dans lequel la substance liante a un poids moléculaire dans la plage de 790 000 à 1 350 000.

8. Papier calque naturel selon la revendication 7, dans lequel la substance liante est la polyvinylpyrrolidone ayant une viscosité définie par une valeur k d'au moins 30, de préférence d'au moins 60, avantageusement d'environ 90.

9. Papier calque naturel selon la revendication 8, dans lequel la quantité de PVP appliquée à la surface du papier calque naturel se situe dans la plage de 0,15 à 0,75 gm⁻², de préférence de 0,4 à 0,7 gm⁻², avantageusement d'environ 0,5 gm⁻².

10. Papier calque naturel selon l'une quelconque des revendications précédentes, dans lequel les substances sont appliquées à la surface du papier calque naturel sous la forme d'une solution aqueuse.

11. Procédé de fabrication d'un papier calque naturel susceptible d'être utilisé avec une table traçante ou une imprimante à jet d'encre en utilisant une encre à base de pigment, ledit papier calque naturel comprenant un papier fabriqué à partir d'une pâte de fibres de cellulose à base de bois qui est mécaniquement traitée pour rendre le papier translucide, caractérisé en ce qu'au moins une surface utile du papier calque naturel est traitée par une combinaison d'une substance cationique soluble dans l'eau et d'une substance liante soluble dans l'eau.

12. Procédé selon la revendication 11, dans lequel le papier calque naturel est traité en appliquant une solution aqueuse de la combinaison de substances à la surface utile du papier, avantageusement en faisant passer le papier calque naturel semi-ouvré à travers un bain de la solution.

13. Procédé d'impression, dans lequel une encre à base de pigment est appliquée à un papier calque naturel avec une table traçante ou une imprimante à jet d'encre, ledit papier calque naturel comprenant un papier fabriqué à partir d'une pâte de fibres de cellulose à base de bois qui est mécaniquement traitée pour rendre le papier translucide, caractérisé en ce qu'au moins une surface utile du papier calque naturel comprend une combinaison d'une substance cationique soluble dans l'eau et d'une substance liante soluble dans l'eau.
